

## UNITED STATES PATENT OFFICE

1,930,765

CARTRIDGE WITH PRIMARY AND  
SECONDARY CHARGES

Josef Meissner, Burbach, Germany

No. Drawing. Application September 29, 1931,  
Serial No. 565,915, and in Germany January 3,  
1931

## 1 Claim. (Cl. 102—9)

The known cartridges as well as their various charges are very deficient and frequently it is the case that the cartridges are not fully fired during the explosions so that shots remain in the blast-hole or detonate incompletely. The measurements of the cartridges and the quantity of their charge are controlled by a syndicate of manufacturers and care has to be taken of the instructions of the mining office with respect to the inner and outer measurements and the diameter of the quick-matches. The cartridges are made in sizes ranging from 1 to 10 and their diameter is very small compared with their length. Hereinafter by way of example a cartridge No. 8 having a diameter of 6.5 to 7 millimetres and a length of 45 millimetres is dealt with.

In the course of time, the charge of the cartridge changed several times and heretofore cartridges were mostly charged either solely with fulminating mercury or with an addition of a fulminating mercury-potassium chlorate mixture. Lately mainly members of the nitro group were employed as secondary charge and a detonating composition, consisting of fulminating mercury and lead-acid, as primary charge. The common charge of cartridge No. 8 consists of:—

0.85 grammie of a member of the nitro group plus 0.4 to 0.5 grammie fulminating mercury, or 30 0.85 grammie of a member of the nitro group plus 0.3 grammie lead-acid.

The measurements of the cartridges are fixed and therefore experiments have been made to produce a greater initial effect by the secondary charge in that tetryl is used in place of trotyl and the secondary charge is more considerably compressed.

Further experiments have been made to produce an increased initial impulse by inwardly pressing the bottom of the cartridge during its manufacture. When firing these cartridges against a lead-plate it has been found that the piercing effect is somewhat greater than in the case of the common cartridges, but the principal aim to produce a positively detonating cartridge is not attained thereby.

Further a cartridge is known in which the bottom part of the nitro-charge is very high, 50 while the top part thereof is pressed-in as usual. If this cartridge is fired against a lead-plate it may appear to be the case that a better effect is attained although the effect is not superior to cartridges of ordinary construction.

By experiments a cartridge-charge has been

discovered which possesses the characteristic of a positive detonation and of a considerably improved initial impulse. The positive detonation takes place only if the primary charge and the secondary charge are separately loaded in the cartridge. The new cartridge is charged in such a way that a primary charge is followed always by a secondary charge, said primary or secondary charge being superposed two or three times according to the length or height of the cartridge. Thus in the event of a case loaded with a treble charge, the individual charges have to be carried out in the following manner: Primary-secondary charge, primary-secondary charge, primary-secondary charge. In view of this division of the whole charge into partial charges it is possible to maintain the initial impulse of the primary charge over the entire height, which is impossible in the case of cartridges with a single secondary—and primary charge. In view thereof the greatest possible quantity of secondary charge is positively initiated and completely detonated with the greatest effect although the smallest possible quantity of primary charge is used (e. g. as limit charge as well as also the practically smallest charge possible). The ideal charge for this kind of cartridge is that the smallest possible quantities of primary charge are combined with the largest quantity of secondary charge, which is permissible as limit charge for the said quantities, and this kind of succession can be repeated in the cartridge as often as desired. In practice this mode of ideal charge cannot be readily carried out, because difficulties arise when loading the secondary charge in quantities which are too small. Owing to the separation of the charge of the cartridges into a number of individual charges in the succession primary-secondary charge, primary-secondary charge and so forth as above described, the following results were obtained during trial shooting with cartridges loaded with a single primary-secondary charge:—

## Old charge I

Charge of the cartridge:—

|                 | Gramme | 10 |
|-----------------|--------|----|
| Trinitrotoluene | 0.85   |    |
| Lead azid       | 0.2    | 10 |

On firing against a lead plate of 5 millimetres, the bottom part of the cartridge with the loaded trinitrotoluene remained on the lead plate in the height of 7 millimetres. Thus only a part 1;

of the trinitrotoluene has been detonated by the 0.2 grammé lead azid.

*New charge I*

Charge of the cartridge:—

|                 | Gramme |
|-----------------|--------|
| Trinitrotoluene | 0.45   |
| Lead azid       | 0.10   |
| Trinitrotoluene | 0.40   |
| Lead azid       | 0.10   |

On firing against a lead plate of 5 millimetres with this charge, the same was readily pierced and this shows the cartridge completely detonated with a high explosive power.

*Old charge II*

Charge of the cartridge:—

|                 | Gramme |
|-----------------|--------|
| Trinitrotoluene | 0.85   |
| Lead azid       | 0.15   |

On firing against a lead plate of 5 millimetres, the bottom part of the cartridge with the loaded trinitrotoluene remained on the lead plate in the height of 7 millimetres. Thus only a partial detonation took place.

*New charge II*

Charge of the cartridge:—

|                 | Gramme |
|-----------------|--------|
| Trinitrotoluene | 0.45   |
| Lead azid       | 0.05   |
| Trinitrotoluene | 0.40   |
| Lead azid       | 0.10   |

The lead plate of 5 millimetres was still readily pierced with this charge, which shows a complete detonation with a high explosive power.

*Old charge III*

Charge of the cartridge:—

|                 | Gramme |
|-----------------|--------|
| Trinitrotoluene | 0.85   |
| Lead azid       | 0.13   |

On firing against the lead plate of 5 millimetres, the copper-case with the loaded trinitrotoluene remained in the height of 19 millimetres, which proves that only the lead azid and a very small quantity of the primary charge detonated during the ignition.

*New charge III*

Charge of the cartridge:—

|                 | Gramme |
|-----------------|--------|
| Trinitrotoluene | 0.45   |
| Lead azid       | 0.03   |
| Trinitrotoluene | 0.40   |
| Lead azid       | 0.10   |

On firing against a lead plate of 5 millimetres it was shown, that the cartridge completely detonated but had not sufficient power to pierce the lead plate. Thus according to the new method, this appears to be the limit charge, while according to the known method the limit charge lies above 0.2 grammé lead azid. It is particularly mentioned, that all cartridges were closed and without inner cap and that the charge was pressed at ordinary pressure. The experiments were carried out under various conditions and always yielded the same result.

I claim:—

A detonating cap comprising a container and primary and secondary charges of explosive material stratified in the container; said primary charge consisting of a mixture of about 0.45 grammé of trinitrotoluene and from 0.03 grammé to 0.10 grammé of lead azid; and said secondary charge consisting of a mixture of about 0.40 grammé of trinitrotoluene and about 0.10 grammé of lead azid.

JOSEF MEISSNER.

80

85

90

95

100

110

115

120

125

130

135

140

145

150